

July 13, 1937.

W. ZETZSCHE ET AL

2,086,888

MANUFACTURE OF A SUBSTITUTE FOR WOOL

Filed Dec. 21, 1935



Walther Zetzsche  
Erich Graumann  
Hermann Faber  
Edmund Stix  
Inventors

By their Attorneys

Hutz and Gorlin

## UNITED STATES PATENT OFFICE

2,086,888

MANUFACTURE OF A SUBSTITUTE  
FOR WOOL

Walther Zetsche, Erich Graumann, Hermann  
Faber, and Edmund Stix, Premnitz, Germany,  
assignors to I. G. Farbenindustrie Aktiengesell-  
schaft, Frankfort-on-the-Main, Germany

Application December 21, 1935, Serial No. 55,664  
In Germany December 24, 1934

5 Claims. (CL. 18—54)

This invention relates to the manufacture of a substitute for wool.

One of its objects is to provide a process for making a substitute for wool. Another object is an apparatus for making a substitute for wool. Further objects will be seen from the detailed specification following hereafter. Reference is made to the accompanying drawing in which the single figure shows diagrammatically an apparatus in accordance with the invention.

A known process of making threads from viscose consists in producing from the viscose xanthate threads, soluble in water or alkali, and then to convert the xanthate thread to a cellulose thread in a second bath. The conversion of the water-soluble thread by means of a mineral acid is performed either on the running thread or on the wound-up thread. For obtaining staple fibers it has been proposed that the xanthate thread spun from the viscose should be cut on the winding device and the mass of threads converted into cellulose fibers by introduction into an acid bath.

In the process of the present invention the xanthate threads spun in known manner into ammonium-sulphate solution, organic acid solution or dilute mineral acid solution are collected from a large number of spinning nozzles to form a thick bundle of several thousand deniers which is then conducted to a cutting machine. The thick bundles are cut into staple and the staple threads are floated in dilute mineral acid whereby a good mechanical loosening of the bundles into separate threads is produced together with a good crimping and at the same time a conversion of the xanthate into cellulose. As the liquid for the floating and the conversion there may advantageously be used sulphuric acid of 1-10 per cent. strength. The acid may be mixed with sodium sulphate or any other of the additions known to be useful in spinning baths for making artificial silk. It is particularly advantageous to use a conversion bath containing, in presence or absence of an acid, an oxidizing agent, such as activin, hypochlorous acid or hydrogen peroxide. The mass of fibers, obtained by the mechanical loosening in the conversion bath and by the conversion and crimping of the xanthate thread cut into the form of staple, is freed from conversion liquor and passed in succession to the various washing and after-treatment baths. In this manner there is obtained in a continuous operation a fleece of a strongly and permanently crimped fiber suitable as a substitute for wool.

The crimping is very stable to the combing action

of the textile machines. In the process of the invention there is no sticking together of separate threads which could not be avoided in the older processes, wherein the xanthate threads were wound on spools or reels before they were cut. 5

A particular mode of the invention is described with reference to the accompanying diagram showing in cross section a suitable apparatus for the purpose. 10

Viscose is spun to xanthate threads in an ammonium sulfate solution of 25 to 30 per cent. strength, containing 5 per cent of sodium sulfate, and the bundles of fibers are united from numerous spinning nozzles to form a thick band *a*. 15 After passing through a draw-off device *b* having the form of rollers driven in opposite directions, the band, without strong pressure, is guided continuously to a cutting machine *c*, whereby it is cut to the desired length of staple. In the cutting 20 operation provision must be made for the shrinking effect on the fiber of the later conversion into cellulose. The cut fibers fall into a trough *d* into which the conversion liquor flows, namely sulfuric acid of 8 per cent. strength containing 25 12 per cent. of sodium sulfate. In order to separate the cut staple length into separate threads the conversion bath is constructed with one or more towers *e*, *e*<sub>1</sub>, having baffles *f* for scattering the fibers. At the lower end of such tower the 30 mass of fibers is received on an endless conveyor sieve *g* and thereby separated from the liquid. This conveyor transports the fleece again upwards in a slanting direction and delivers it into a further tower *e*<sub>2</sub>, also having baffle plates *f*; here 35 the fibers are washed free from conversion liquor by water. The threads are passed in similar manner through all the necessary treatment baths. At the end of each conveyor sieve the fibrous mass is passed between pressure rollers *h* in order to 40 express the absorbed liquid. Finally the fibers pass on to the conveyor bands of a drying cupboard *i*. Instead of the after-treatment of the fibers in scattering towers in the manner described, there may be used for the after-treatment 45 a powerful sprinkling with the various liquids on the conveyor sieves. Or such a sprinkling may be supplemental to the treatment in scattering towers.

The treating liquors are collected in troughs *k* 50 under the conveyor sieves whence they are discharged to tanks *l* where they are adjusted to the original concentration and returned to the towers by means of pumps *m*.

The product of the invention is a staple fiber 55

in the form of a fleece of good wool-like crimping, which is very suitable for spinning.

What we claim is:

1. A process of producing a substitute for wool which comprises precipitating viscose in the form of threads to cellulose xanthogenate, assembling the threads to endless fiber bands of high total titer, cutting the fiber bands into staple, and mechanically opening the staple threads by means of an acid liquid while simultaneously decomposing the xanthogenate to cellulose hydrate, after-treating the formed fleece of opened fibers, and drying the fleece.
2. A process of producing a substitute for wool which comprises precipitating viscose in the form of threads to cellulose xanthogenate, assembling the threads to endless fiber bands of high total titer, cutting the fiber bands into staple, and mechanically opening the staple threads by means of an acid liquid containing a salt, while simultaneously decomposing the xanthogenate to cellulose hydrate, after-treating the formed fleece of opened fibers, and drying the fleece.
3. A process of producing a substitute for wool which comprises precipitating viscose in the form of threads to cellulose xanthogenate, assembling the threads to endless fiber bands of high total titer, cutting the fiber bands into staple, and mechanically opening the staple threads by means of an acid liquid containing an oxidizing agent while simultaneously decomposing the xanthogenate to cellulose hydrate, after-treating the formed fleece of opened fibers, and drying the fleece.
4. A process of producing a substitute for wool which comprises precipitating viscose in the form of threads to cellulose xanthogenate, assembling the threads to endless fiber bands of high total titer, cutting the fiber bands into staple, and mechanically opening the staple threads by means of a liquid containing 1 to 10 per cent of sulfuric acid while simultaneously decomposing the xanthogenate to cellulose hydrate, after-treating the formed fleece of opened fibers, and drying the fleece.
5. A process of producing a substitute for wool which comprises precipitating viscose in the form of threads to cellulose xanthogenate, assembling the threads to endless fiber bands of high total titer, cutting the fiber bands into staple, and mechanically opening the staple threads by means of sulfuric acid of 8 per cent strength containing 12 per cent of sodium sulfate while simultaneously decomposing the xanthogenate to cellulose hydrate, after-treating the formed fleece of opened fibers, and drying the fleece.

WALTHER ZETZSCHE.  
ERICH GRAUMANN.  
HERMANN FABER.  
EDMUND STIX.

30